

# UNITED STATES PATENT OFFICE.

WILLIAM S. NUTTER, OF SANFORD, MAINE, ASSIGNOR TO GOODALL WORSTED COMPANY, OF SANFORD, MAINE, A CORPORATION OF MAINE.

## FABRIC.

1,252,018.

Specification of Letters Patent.

Patented Jan. 1, 1918.

No Drawing.

Application filed March 28, 1916. Serial No. 87,322.

*To all whom it may concern:*

Be it known that I, WILLIAM S. NUTTER, a citizen of the United States, residing at Sanford, county of York, State of Maine, 5 have invented an Improvement in Fabric, of which the following description is a specification.

This invention relates to fabrics having embodied therein either as the warp or the 10 weft thread a yarn made partially at least from the fleece of the Angora goat. As is well known, the Angora fleece contains fibers of two different characters, that is, a white fiber with comparatively little life and which 15 will not take dye readily, and another fiber with considerable life which will readily take the dye. The first-named white fiber, and that which will not readily take the dye, is known to the trade as "kemp" and will 20 be thus hereinafter referred to. These kemp fibers are usually rather coarse fibers somewhat larger than the other fibers which take the dye readily.

A yarn which is spun from tops from the 25 Angora fleece containing the kemp fibers is more or less streaky in appearance even when it is undyed because the kemp fibers are of such a character that they are readily distinguished from the other fibers of the 30 yarn.

It has heretofore been proposed to manufacture an undyed fabric, the weft yarn of 35 which has the so-called kemp fibers therein and is woven into the cloth in its natural color. A cloth made in this way is illustrated and described in my Patent No. 1,131,259, March 9, 1915, said cloth having a variegated warp thread, the purpose of 40 which is to break up the streaky appearance of the kemp fibers in the weft yarn.

The natural color of the mohair fleece is a 45 very light tan, almost white, and a cloth made from the mohair yarn in its natural color will consequently be almost white. Cloth of this nature has proved to be extremely acceptable for the manufacture of summer clothing, but one objection to a light-colored or white cloth for summer suits is that it 50 readily shows the soil and requires constant laundrying to be kept in an immaculate condition. A darker-colored fabric is not subjected to this disadvantage because slight soiling thereof is not visible.

55 My present invention has for its object to provide a mohair fabric of the general type described in my above-mentioned patent and which has all the advantages thereof so far as coolness and wearing qualities are concerned, but which can be made of a considerably darker shade than the natural color of the Angora fleece without developing any streaky appearance due to the presence of the kemp fibers. I propose to accomplish this object by using for either the weft or the 60 warp of the fabric, but preferably for the weft, a yarn spun from a mixture of the undyed mohair tops having the kemp fibers therein and a fibrous material of a darker color. In thus mixing the darker material 65 with the mohair material, care must be taken not to use a sufficient amount of the darker material to cause the kemp fibers of the mohair to become prominent by contrast in the completed fabric. The proportion of 70 darker material which can be used depends upon the nature thereof and its color. A less quantity of a relatively-dark material 75 can be used than of a relatively-lighter material. The mixing of the darker material 80 with the mohair material tends to bring the kemp fibers into view by contrast and thus augments the streaky appearance of the yarn and of the fabric made therefrom due to the presence of the kemp fibers. A certain proportion 85 of darker material, however, can be successfully used without making the kemp fibers prominently visible. Any suitable material may be used for thus darkening the shade of the mohair yarn, such, for instance, 90 as silk, alpaca, wool, cotton, camel's hair, etc. The darkening or coloring material of whatever type or shade may be mixed or twisted, or otherwise incorporated with the mohair or Angora fleece fibers before or during 95 the combing operation, or in any of the operations of manufacture up to and including the operation of spinning, so that whenever the yarn is finally spun from the roving it is made partly from the fleece of the 100 Angora goat containing the kemp fibers, and partly from the material used for darkening the shade thereof. The yarn thus formed is used for either the weft or the warp thread of the fabric to be made, but will preferably 105 be used for the weft. For the warp, I propose to use a yarn preferably having a variegated coloring throughout its length as described in the before-mentioned patent. This can be provided for by twisting together two 110

strands of different color. The character of the two colors which are used in the two strands of the warp thread will vary somewhat, depending on the character of the cloth to be made. The purpose of the variegated warp thread is to break up the streaky appearance due to the presence of the kemp fibers in the weft thread, all as set forth in the above-mentioned patent.

10 The darkening of the shade or coloring of the weft thread by the use of a certain proportion of the fibrous material of darker shade tends to make the kemp fibers more prominent by contrast, but a certain proportion 15 of this dark fibrous material mixed with the Angora tops in the formation of the weft thread will not show up the kemp fibers to such an extent as to produce a streakiness that is not broken up by the variegated warp 20 thread. The proportion of darkening fibrous material which is used in the weft thread, therefore, must have relation to the shade of such fibrous material and must always be so proportioned that the presence of this darker 25 fibrous material in the weft yarn does not cause the kemp fibers to become prominent by contrast. The presence of this darkening fibrous material in the weft yarn gives a darker tone or shade to the fabric which is 30 a desirable feature, but by properly proportioning the amount which is used, the unde-

sirable streaky appearance due to the presence of the kemp threads is not apparent.

My invention, therefore, resides in mixing with the Angora tops having the kemp fibers 35 therein a fibrous material of a darker shade than the top and in such proportions as to appreciably darken the shade of the fabric without, however, causing the kemp fibers to become prominent by contrast. 40

I claim:

A woven fabric comprising interwoven warp and weft threads, the weft thread being made by spinning together the undyed fibers of the Angora fleece including the 45 kemp fibers thereof and a fibrous material having a darker shade than said Angora fleece fibers, and the warp being a variegated thread which operates to break up the streaky appearance due to the presence of 50 the kemp fibers in the weft, the amount of fibrous material of darker shade which is used in the weft having such relation to the variegated warp and the kemp fibers as to 55 appreciably darken the shade of the fabric without, however, destroying the effect of the variegated warp in breaking up the streaky appearance due to the presence of the kemp fibers.

In testimony whereof, I have signed my 60 name to this specification.

WILLIAM S. NUTTER.

Copies of this patent may be obtained for five cents each, by addressing the "Commissioner of Patents, Washington, D. C."